# EUROPEAN PATENT SPECIFICATION

(11) **EP 0 661 588 B1**
(45) Date of publication and mention of the grant of the patent: **20.10.1999**
(21) Application number: 94420363.7
(22) Date of filing: 20.12.1994
(51) Int. Cl.: G03C 1/005, G03C 7/388

(54) **Color photographic element**
Farbphotographisches Element
Elément photographique couleur

(30) Priority: 30.12.1993 US 175821; 30.12.1993 US 175824
(43) Date of publication of application: 05.07.1995
(73) Proprietor: EASTMAN KODAK COMPANY, Rochester, New York 14650-2201 (US)
(72) Inventor: Chari, Krishnan, c/o EASTMAN KODAK COMPANY, Rochester, New York 14650-2201 (US); Miller, David Darrell c/o EASTMAN KODAK COMPANY, Rochester, New York 14650-2201 (US)
(74) Representative: Parent, Yves

(56) References cited:
- EP-A- 0 276 319
- EP-A- 0 560 457
- GB-A- 540 366
- US-A- 2 269 158

## Description

### Background of the Invention

This invention relates to photography, and in particular to color photographic elements having improved image stability and to methods for preparing stabilized dispersions of photographically useful compounds (PUCs) and to stabilized photographic dispersions.

It is well known that yellowing, dye fade and thermal pinking are major concerns in the image stability of color prints. Over the years improvement in image stability has been achieved by introducing new couplers having a better resistance to dye fade and yellowing and also by introducing more efficient image stabilizers. However, in spite of this, the present level of stability is not considered satisfactory.

It has been known for a number of years that both fading of magenta and yellow image dyes and yellowing of residual magenta coupler are exacerbated by the presence of oxygen. This has led to the search for antioxidants and oxygen barriers. For example, improvements in dye fade and yellowing may be obtained by laminating a color print using polyethylene terephthalate. However, lamination is an expensive and laborious process.

Couplers and other PUCs are usually incorporated into photographic materials by dissolving the PUC in a high boiling organic solvent, optionally with a low boiling water immiscible auxiliary solvent, and then dispersing the resulting solution as an oil phase in an aqueous medium which generally contains a hydrophilic colloid, such as gelatin. To ensure thin layers and good physical performance of the photographic element, only very low levels of such solvents are used. As a result of low solvent levels, the PUCs are susceptible to crystallization prior, during, and after coating. Such crystallization causes difficulties both in the manufacture and in the use of the photographic element.

US 2,269,158 and GB 540,366 are directed to photographic elements including rosin compounds and photographic color formers in order to prevent wandering of color couplers.

EP 560,457 provides a photographic print having a stability of the developed pivalylacetanilide yellow coupler by adding into a conventional dispersion a polyalkylene surface active agent.

Several recent patents suggest that improvements in image stability may be obtained by incorporating hydrophobic polymers in the oil phase of such dispersions. See for example, U.S Patents Nos. 4,710,454; 4,857,449; 5,001,045; 5,006,453; 5,043,255; 5,047,316; 5,055,386 and EP 276,319. Many of these polymers have good oxygen insulating properties in the glassy state. However, the presence of high molecular weight polymers generally results in very high viscosities for the oil phase leading to large particle size and a subsequent decrease in dye density. The latter may be circumvented by using large amounts of a low boiling auxiliary solvent, such as ethyl acetate, which is then removed by evaporation, but this raises serious environmental concerns and adds additional expense. Attempts have also been made to solve PUC crystallization problems. For example, U.S. 3,700,454 to Sakamoto et al. discloses the incorporation of fragments of the PUC molecule in the PUC dispersion to minimize PUC crystallization. Unfortunately, we have found that this method frequently requires high levels of the fragment to be effective, thus raising the cost to manufacture the photographic element and increasing the thickness of the layer containing the PUC dispersion. In addition, these materials are often very expensive and not generally commercially available.

### Problem to be Solved by the Invention

There is therefore a need for materials that can inhibit crystallization of PUCs when incorporated in the oil phase of dispersions and improve image stability of photographic elements without the disadvantages encountered with prior art approaches.

### Summary of the Invention

One aspect of this invention comprises a silver halide color photographic element as claimed in Claim 1.

A further aspect of this invention comprises a method of improving the image stability of a silver halide color photographic element comprising at least one light sensitive silver halide emulsion layer comprising a hydrophilic colloid phase and an oily-phase comprising dispersed particles of a ballasted photographic coupler and an organic solvent, which method comprises incorporating in said oily-phase at least one non-color forming, oil-soluble, monomeric or oligomeric organic compound as recited in Claim 1.

### Advantageous Effects of the Invention

This invention provides a silver halide based color photographic element having excellent image stability in terms of yellowing, dye fade and thermal pinking. Additionally, undesired crystallization of a PUC in a photographic dispersion is inhibited by incorporating a non-color forming, oil-soluble, monomeric, or oligomeric organic compound into the dispersion. Very low levels of such compounds are effective, thus avoiding the disadvantages of the fragment approach described above. The preferred rosin compounds and oil-soluble sucrose esters for use in the present invention are also very inexpensive and readily available. Another advantage to using low levels of the rosin compounds or oil-soluble sucrose esters is that low cost photographic elements can be produced with no adverse effects on PUC performance. Finally, many of these compounds are natural products and have low toxicity.

### Detailed Description of the Invention

In accordance with preferred embodiments of this invention, a low molecular weight organic glass is incorporated into a layer of a color photographic element. In especially preferred embodiments of the invention, photographic dispersions with improved stability to crystallization are prepared by incorporating low levels of at least one low molecular weight organic glass in the mixture of high boiling organic solvent(s) and PUC(s) prior to forming the dispersion.

In this specification, the term "low molecular weight organic glass" refers to any non-color forming, oil-soluble, monomeric or oligomeric organic compound having a glass transition temperature between 0°C and 150°C, preferably 0°C and 100°C. The organic glass preferably has a molecular weight below about 1000, preferably below about 500. Furthermore, the organic glass should be miscible with organic solvents commonly used in preparing photographic elements, such as dibutyl phthalate or tricresyl phosphate.

Preferred organic glass materials for use in this invention are oil soluble gums, rosins, natural resins and their derivatives, esters of lactose, oil soluble galactomannons, glycol esters, naturally occurring esters of oligomeric glycol esters, alkylbetaglycoside ethers, where the alkyl group contains at least 8 carbon atoms, and water-insoluble derivatives of sucrose, including sucrose esters, and polyesters, esterified sugars or sugar alcohols, such as erythritol, xylitol, sorbitol, glucose or sucrose, esterified with at least four fatty acid groups, such as caprylic, capric, lauric myristic, myristoleic, palmitic, palmitoleic, stearic, oleic, ricinoleic, linoleic, linolenic, eleostearic, etc.; and esterified alkoxylated sugar or sugar alcohols esterified with at least four fatty acid groups. Oil-soluble gums, rosins, natural resins and their derivatives including, for example, rosin acids, such as abietic acid, neoabietic acid, palustric acid, pimaric acid, isopimaric acid, levopimaric acid, hydrogenated rosin acids; and salts, esters and amides of such acids; natural resins, such as damar, East India (pale or black), pine gum, pontiniak, Manila, elemi, yacca (accroides), gilsonite, gum rosin, wood rosin, and tall oil rosin. Many rosin derivatives are commercially available from Hercules, Incorporated of Wilmington Delaware under the trade marks Foral®, Poly-Pale®, Staybellite®, Pamite® and numerous others.

One class of preferred organic glass materials comprises oil-soluble sucrose esters, such as sucrose octaacetate. Another class of preferred organic glass materials comprises rosin and derivatives thereof.

The mechanism by which crystallization of PUCs, yellowing, dye fade and thermal pinking is inhibited is not entirely understood. While it is believed that the effectiveness of the material added is due to its glassy characteristics, it is also contemplated that the particular effectiveness of rosin and derivatives thereof might be due to chemical characteristics or other physical properties.

In certain preferred embodiments of the invention, rosin, or derivative thereof, is incorporated into a photographic dispersion of a ballasted photographic coupler in a photographic element. Preferred rosin derivatives have the structure: where A is a saturated or unsaturated alkyl group of 1-10 carbons and B is a hydrogen atom or a saturated or unsaturated alkyl group of 1-10 carbons and n is 0 or 1. Bonds between the numbered corners of the ring structure can be single or double bonds.

Specific examples of rosins of the above formula which can be utilized in the present invention are given below. It is understood that this list is representative only, and not meant to be exclusive.

| Compound | A | (B)ₙ | double bonds | name |
|---|---|---|---|---|
| R-A | isopropyl | n=0 | 2-3, 4-5 | abietic acid |
| R-B | isopropyl | n=0 | 1-2, 3-4 | levopimaric acid |
| R-C | isopropyl | n=0 | 2-3, 4-6 | palustric acid |
| R-D | isopropyl | n=0 | 1-2, 3-4, 6-7 | dehydroabietic acid |
| R-E | isopropyl | H (n=1) | none | tetrahydroabietic acid |
| R-F | isopropylidene | H (n=1) | 3-4 | neoabietic acid |
| R-G | vinyl | methyl (n=1) | 3-4 | pimaric acid |
| R-H | vinyl | methyl (n=1) | 4-5 | isopimaric acid |
| R-I | vinyl | methyl (n=1) | 4-6 | isopimaric acid |

Particularly preferred is abietic acid which has the structural formula: R-A (abietic acid) Tg∼65°C

Color photographic elements are typically multilayer elements comprising a plurality of layers coated on a support, at least one of which is light sensitive. The organic glass may be incorporated into any layer of the photographic element. The organic glass is incorporated into a layer by forming a dispersion of the organic glass and a high boiling organic solvent, such as dibutyl phthalate or tricresyl phosphate, and optionally a PUC, in an aqueous medium, preferably containing a hydrophilic colloid. The dispersion is then coated onto a support to form a layer. In a preferred embodiment, the invention improves upon conventional dispersions of photographic materials, such as couplers, UV absorbers, oxidized developer scavengers, etc., by incorporating small amounts (0.01% to 100%, by weight, based on the weight of the PUC, preferably 1% to 50% and most preferably 5% to 30% ) of an organic glass (or rosin compound) into the dispersed organic phase.

It is to be understood that mixtures of organic glass compounds and/or rosin or rosin derivatives can be used. Preferably the amount of organic glass and/or rosin or rosin derivative used in a photographic element of this invention is between about 0.001 to about 1.72 g/m².

Below are listed representative photographically useful compounds, high boiling solvents and auxiliary solvents. Typically, the PUC(s), high boiling solvent(s), and organic glass (or rosin derivative) are codissolved and then dispersed in aqueous surfactant or aqueous gelatin/surfactant aqueous solutions. Dispersal can be accomplished using high shear mixing, a colloid mill, a microfluidizer, a homogenizer, or ultrasonic energy. Other compounds in the aqueous phase, such as polymeric thickeners and stabilizers are also acceptable. To aid codissolution and/or achieve low particle size, an low-boiling, auxiliary solvent compatible with the photographic material and the hydrophobic material can be used. Auxiliary solvents such as ethyl acetate and butoxyethoxy ethyl acetate are well known in the photographic literature, and are removed after dispersion making by evaporation, washing, or dialysis. Also listed below are typical auxiliary solvents used in photographic dispersion making.
A. Illustrative photographically useful compounds
   1. Ballasted Couplers
      a. 2 equivalent
      b. 4 equivalent
      c. cyan
      d. magenta
      e. yellow
      f. DI(A)R
      g. BARC
   2. UV absorbers
   3. Oxidized Developer Scavengers
   4. Optical Brighteners
   5. Incorporated Developers
   6. Antifogging Agents
B. Illustrative high boiling solvents
   n-Hexylphenylcarbinol; 2-(*p*-tert-butylphenoxy)-ethanol; Acetyl n-butyl aniline; Acetyl methyl *p*-toluidine; Benzoyl piperdine; N-n-amylphthalimide; N-n-amyl succinimide; N-2-cyanobutylphthalimide; N,N-diethyl-dodecanamide; N,N-dimethyl dodecanamide; N,N-dipropyl dodecanamide; di-tert-amyl phenol; phenoxy toluene; bis-ethylhexyl sulfoxide; acetyl tributyl citrate; tributyl citrate; ethylhexyl hydroxy benzoate; ethylhexyltoluene sulfonamide; undecyl alcohol; diethyl sebacate; dimethyl sebacate; ethyl phenylacetate; triethyl citrate; 1,4-cyclohexylenedimethylene bis(2-ethylhexanoate); Ethyl N,N-di-n-butyl carbamate; Ethyl N-phenyl carbamate; Tetrahydrofurfuryl benzoate; Tetrahydrofurfuryl succinate; Ethylbenzyl malonate; diethyl phthalate; dibutyl phthalate; dipentyl phthalate; diisoamyl phthalate; dibenzyl phthalate; dimethoxyethyl phthalate; diethoxyethyl phthalate; dibutoxyethyl phthalate; ethyl
   naphthoate; methyl methoxy benzoate; butyl methoxy benzoate; naphthyl acetate; methyl phthalylethyl glycollate; butyl phthalybutyl glycollate; resorcinol diacetate; hexyl benzoate; benzophenone; dicholorbenzophenone; methoxy acetophenone; acetophenone; 2,4-dihydroxy valerophenone; *p*-sec-amylbenzophenone; triphenyl phosphate; tricresylphosphate; diphenyl mono-*p*-tert-butylphenyl phosphate; monophenyl di-p-tert-butylphenyl phosphate; diphenyl mono-o-chlorophenyl phosphate; monophenyl di-o-chlorophenyl phosphate; tri-*p*-tert-butylphenyl phosphate; tri-o-phenylphenyl phosphate; di-*p*-tert. butylphenyl mono (5-tert-butyl-2-phenylphenyl) phosphate; *p*-toluenesulfonyl methyl o-toluidine; p-toluenesulfonyl dimethylamide; *p,p'*-di-n-amylbenzenesulfonanilide; ρ-toluenesulfonyl di-n-butyl amide; n-butylsulfone; iso-amyl sulfone; N,N'-diethyl-N,N'-diphenyl urea; N,N'-di-n-butyl urea
C. Illustrative auxiliary solvents
   methyl isobutyl ketone; methyl acetate; 2-methyl tetrahydrofuran; isobutyl acetate; 2-ethoxyethyl acetate; 2-(2-butoxyethoxy)ethyl acetate; 4-methyl-2-pentanol; ethyl acetate; diethyl carbitol; triethyl phosphate; cyclohexanone; 2-benzyloxyethanol; 2-(2-ethoxyethoxy)ethyl acetate; methylene chloride; 1,1,2-trichloroethane; 1,2-dichloropropane

An oil-soluble polymer may also be incorporated into the photographic element. The oil-soluble polymer is added to an oil phase of a photographic dispersion used in the preparation of the element. In preferred embodiments the oil-soluble polymer is added to the same dispersion as the organic glass (or rosin or rosin derivative). Illustrative oil-soluble polymers are disclosed in above noted U.S. Patents Nos. 4,710,454; 4,857,449; 5,001,045; 5,006,453; 5,043,255; 5,047,316; and 5,055,386.

Typically, color photographic elements comprise at least one layer sensitive to red light and comprising a silver halide emulsion and a ballasted cyan dye forming coupler, at least one layer sensitive to green light and comprising a silver halide emulsion and a ballasted magenta dye forming coupler and at least one layer sensitive to blue light and comprising a silver halide emulsion and a ballasted yellow dye forming coupler. The light sensitive layers can be in any desired order. The organic glass may be incorporated in the dispersed oil phase of one of said light sensitive layers or in a non-light sensitive layer of the photographic element, for example an interlayer positioned between light sensitive layers, a filter layer, a subbing layer, an antihalation layer, an overcoat layer, or the like.

When used in a light sensitive layer, the organic glass material is preferably incorporated as an addendum to the oil phase of a dispersion of one of the couplers, preferably the magenta or yellow coupler. In this case, the organic glass, coupler and high boiling permanent solvent are heated to form a solution which is then added to an aqueous medium containing a hydrophilic colloid. This dispersion is then added to the silver halide emulsion prior to coating onto a support in the manufacture of the photographic element.

If desired, the photographic element can be used in conjunction with an applied magnetic layer as described in Research Disclosure, November 1992, Item 34390 published by Kenneth Mason Publications, Ltd., Dudley Annex, 12a North Street, Emsworth, Hampshire P010 7DQ, ENGLAND.

In the following discussion of suitable materials for use in the elements of this invention, reference will be made to Research Disclosure, December 1989, Item 308119, available as described above, which will be identified hereafter by the term "Research Disclosure." The contents of the Research Disclosure, including the patents and publications referenced therein, are incorporated herein by reference, and the Sections hereafter referred to are Sections of the Research Disclosure.

The silver halide emulsions employed in the elements of this invention can be either negative-working or positive-working. Suitable emulsions and their preparation as well as methods of chemical and spectral sensitization are described in Sections I through IV. Color materials and development modifiers are described in Sections V and XXI. Vehicles are described in Section IX, and various additives such as brighteners, antifoggants, stabilizers, light absorbing and scattering materials, hardeners, coating aids, plasticizers, lubricants and matting agents are described , for example, in Sections V, VI, VIII, X, XI, XII, and XVI. Manufacturing methods are described in Sections XIV and XV, other layers and supports in Sections XIII and XVII, processing methods and agents in Sections XIX and XX, and exposure alternatives in Section XVIII.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocyclyl, sulfonamido, mercaptotetrazole, benzothiazole, mercaptopropionic acid, phosphonyloxy, arylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in U.K. Patents and published application Nos. 1,466,728, 1,531,927, 1,533,039, 2,006,755A and 2,017,704A, the disclosures of which are incorporated herein by reference.

Image dye-forming couplers may be included in the element such as couplers that form cyan dyes upon reaction with oxidized color developing agents which are described in such representative patents and publications as: U.S. Pat. Nos. 2,772,162, 2,895,826, 3,002,836, 3,034,892, 2,474,293, 2,423,730, 2,367,531, 3,041,236, 4,883,746 and "Farbkuppler-eine LiteratureUbersicht," published in Agfa Mitteilungen, Band III, pp. 156-175 (1961). Preferably such couplers are phenols and naphthols that form cyan dyes on reaction with oxidized color developing agent.

Couplers that form magenta dyes upon reaction with oxidized color developing agent are described in such representative patents and publications as: U.S. Pat. Nos. 2,600,788, 2,369,489, 2,343,703, 2,311,082, 3,152,896, 3,519,429, 3,062,653, 2,908,573 and "Farbkuppler-eine LiteratureUbersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents.

Couplers that form yellow dyes upon reaction with oxidized and color developing agent are described in such representative patents and publications as: U.S. Pat. Nos. 2,875,057, 2,407,210, 3,265,506, 2,298,443, 3,048,194, 3,447,928 and "Farbkuppler-eine LiteratureUbersicht," published in Agfa Mitteilungen, Band III, pp. 112-126 (1961). Such couplers are typically open chain ketomethylene compounds.

It may be useful to use a combination of couplers any of which may contain known ballasts or coupling-off groups such as those described in U.S. Patent 4,301,235; U.S. Patent 4,853,319 and U.S. Patent 4,351,897. The coupler may also be used in association with "wrong" colored couplers (e.g. to adjust levels of interlayer correction) and, in color negative applications, with masking couplers such as those described in EP 213.490; Japanese Published Application 58-172,647; U.S. Patent 2,983,608; German Application DE 2,706,117C; U.K. Patent 1,530,272; Japanese Application A-113935; U.S. Patents 4,070,191 and 4,273,861; and German Application DE 2,643,965. The masking couplers may be shifted or blocked.

Typical couplers and stabilizers that can be used in the elements of this invention are shown below.

### Magenta Couplers

### Yellow Couplers

### Cyan Couplers

### Stabilizers

The invention materials may also be used in association with materials that accelerate or otherwise modify the processing steps e.g. of bleaching or fixing to improve the quality of the image. Bleach accelerator releasing couplers such as those described in EP 193,389; EP 301,477; U.S. 4,163,669; U.S. 4,865,956; and U.S. 4,923,784, may be useful. Also contemplated is use of the compositions in association with nucleating agents, development accelerators or their precursors (UK Patent 2,097,140; U.K. Patent 2,131,188); electron transfer agents (U.S. 4,859,578; U.S. 4,912,025); antifogging and anti color-mixing agents such as derivatives of hydroquinones, aminophenols, amines, gallic acid; catechol; ascorbic acid; hydrazides; sulfonamidophenols; and non color-forming couplers.

For example, in a color negative element, the materials of the invention may replace or supplement the materials of an element comprising a support bearing the following layers from top to bottom:
(1) one or more overcoat layers containing ultraviolet absorber(s);
(2) a two-coat yellow pack with a fast yellow layer containing "Coupler 1": Benzoic acid, 4-chloro-3-((2-(4-ethoxy-2,5-dioxo-3-(phenylmethyl)-1-imidazolidinyl)-3-(4-methoxyphenyl)-1,3-dioxopropyl)amino)-, dodecyl ester and a slow yellow layer containing the same compound together with "Coupler 2": Propanoic acid, 2-[[5-[[4-[2-[[[2,4-bis(1,1-dimethylpropyl)phenoxy]acetyl]amino]-5-[(2,2,3,3,4,4,4-heptafluoro-1-oxobutyl)amino]-4-hydroxyphenoxy]-2,3 -dihydroxy-6-[(propylamino)carbonyl ]phenyl]thio)-1,3,4-thiadiazol-2-yl]thio]-,methyl ester and "Coupler 3": 1-((dodecyloxy)carbonyl) ethyl(3-chloro-4-((3-(2-chloro-4-((1-tridecanoylethoxy) carbonyl)anilino)-3-oxo-2-((4)(5)(6)-(phenoxycarbonyl)-1H-benzotriazol-1-yl)propanoyl)amino))benzoate;
(3) an interlayer containing fine metallic silver;
(4) a triple-coat magenta pack with a fast magenta layer containing "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-,"Coupler 5": Benzamide, 3-((2-(2,4-bis(1,1-dimethylpropyl)phenoxy)-1-oxobutyl)amino)-N-(4',5'-dihydro-5'-oxo-1'-(2,4,6-trichlorophenyl) (1,4'-bi-lH-pyrazol)-3'-yl)-,"Coupler 6": Carbamic acid, (6-(((3-(dodecyloxy)propyl) amino)carbonyl)-5-hydroxy-1-naphthalenyl)-, 2-methylpropyl ester , "Coupler 7": Acetic acid, ((2-((3-(((3-(dodecyloxy)propyl)amino) carbonyl)-4-hydroxy-8-(((2-methylpropoxy)carbonyl) amino)-1-naphthalenyl) oxy)ethyl)thio)-, and "Coupler 8 " Benzamide, 3-((2-(2,4-bis(1,1-dimethylpropyl) phenoxy)-1-oxobutyl)amino)-N-(4,5-dihydro-4-((4-methoxyphenyl) azo)-5-oxo-1-(2,4,6-trichlorophenyl)-1H-pyrazol-3-yl)-; a mid-magenta layer and a slow magenta layer each containing "Coupler 9": a ternary copolymer containing by weight in the ratio 1:1:2 2-Propenoic acid butyl ester, styrene, and N-[1-(2,4,6-trichlorophenyl)-4,5-dihydro-5-oxo-lH-pyrazol-3-yl]-2-methyl-2-propenamide; and "Coupler 10": Tetradecanamide, N-(4-chloro-3-((4-((4-((2,2-dimethyl-1-oxopropyl) amino)phenyl)azo)-4,5-dihydro-5-oxo-1-(2,4,6-trichlorophenyl)-lH-pyrazol-3-yl )amino)phenyl)-, in addition to Couplers 3 and 8;
(5) an interlayer;
(6) a triple-coat cyan pack with a fast cyan layer containing Couplers 6 and 7; a mid-cyan containing Coupler 6 and "Coupler 11": 2,7-Naphthalenedisulfonic acid, 5-(acetylamino)-3-((4-(2-((3-(((3-(2,4-bis(1,1-dimethylpropyl)phenoxy) propyl)amino)carbonyl)-4-hydroxy-1-naphthalenyl) oxy)ethoxy)phenyl) azo) -4-hydroxy-, disodium salt; and a slow cyan layer containing Couplers 2 and 6;
(7) an undercoat layer containing Coupler 8; and
(8) an antihalation layer.

In a color paper format, the materials of the invention may replace or supplement the materials of an element comprising a support bearing the following layers from top to bottom:
(1) one or more overcoats;
(2) a cyan layer containing "Coupler 1": Butanamide, 2-(2,4-bis(1,1-dimethylpropyl)phenoxy)-N-(3,5-dichloro-2-hydroxy-4-methylphenyl)-, "Coupler 2": Acetamide, 2-(2,4-bis(1,1-dimethylpropyl)phenoxy)-N-(3,5-dichloro-2-hydroxy-4-, and UV Stabilizers: Phenol, 2-(5-chloro-2H-benzotriazol-2-yl)-4,6-bis(1,1-dimethylethyl)-;Phenol, 2-(2H-benzotriazol-2-yl)-4-(1,1-dimethylethyl)-; Phenol, 2-(2H-benzotriazol-2-yl)-4-(1,1-dimethylethyl)-6-(1-methylpropyl)-; and Phenol, 2-(2H-benzotriazol-2-yl)-4,6-bis(1,1-dimethylpropyl)-and a poly(t-butylacrylamide) dye stabilizer;
(3) an interlayer;
(4) a magenta layer containing "Coupler 3": Octanamide, 2-[2,4-bis(1,1-dimethylpropyl)phenoxy]-N-[2-(7-chloro-6-methyl-lH-pyrazolo[1,5-b] [1,2, 4] triazol-2-yl)propyl]- together with 1,1'-Spirobi(lH-indene), 2,2',3,3 '-tetrahydro-3,3,3',3'-tetramethyl-5,5',6,6'-tetrapropoxy-;
(5) an interlayer; and
(6) a yellow layer containing "Coupler 4": 1-Imidazolidineacetamide, N-(5-((2-(2,4-bis(1,1-dimethylpropyl)phenoxy)-1-oxobutyl)amino)-2-chlorophenyl)-alpha.- (2,2-dimethyl-1-oxopropyl)-4-ethoxy-2,5-dioxo-3-(phenylmethyl)-.

In a reversal format, the materials of the invention may replace or supplement the materials of an element comprising a support bearing the following layers from top to bottom:
(1) one or more overcoat layers;
(2) a nonsensitized silver halide containing layer;
(3) a triple-coat yellow layer pack with a fast yellow layer containing "Coupler 1": Benzoic acid, 4-(1-(((2-chloro-5-((dodecylsulfonyl)amino)phenyl) amino)carbonyl)-3,3-dimethyl-2-oxobutoxy)-, 1-methylethyl ester; a mid yellow layer containing Coupler 1 and "Coupler 2": Benzoic acid, 4-chloro-3-[[2-[4-ethoxy-2,5-dioxo-3-(phenylmethyl)-1-imidazolidinyl] -4,4-dimethyl-1,3-dioxopentyl] amino]-, dodecylester; and a slow yellow layer also containing Coupler 2;
(4) an interlayer;
(5) a layer of fine-grained silver;
(6) an interlayer;
(7) a triple-coated magenta pack with a fast magenta layer containing "Coupler 3": 2-Propenoic acid, butyl ester, polymer with N-[1-(2,5-dichlorophenyl)-4,5-dihydro-5-oxo-1H-pyrazol-3-yl]-2-methyl-2-propenamide; "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-; and "Coupler 5": Benzamide, 3-(((2,4-bis(1,1-dimethylpropyl)phenoxy)acetyl)amino)-N-(4,5-dihydro-5-oxo-1-(2,4,6-trichlorophenyl)-1H-pyrazol-3-yl)-; and containing the stabilizer 1,1'-Spirobi(1H-indene), 2,2',3,3'-tetrahydro-3,3,3',3'-tetramethyl-5,5',6,6'-tetrapropoxy-; and in the slow magenta layer Couplers 4 and 5 with the same stabilizer;
(8) one or more interlayers possibly including fine-grained nonsensitized silver halide;
(9) a triple-coated cyan pack with a fast cyan layer containing "Coupler 6": Tetradecanamide, 2-(2-cyanophenoxy)-N-(4-((2,2,3,3,4,4,4-heptafluoro-1-oxobutyl)amino)-3-hydroxyphenyl)-; a mid cyan containing "Coupler 7": Butanamide, N-(4-((2-(2,4-bis(1,1-dimethylpropyl)phenoxy)-1-oxobutyl)amino)-2-hydroxyphenyl)-2,2,3,3,4,4,4-heptafluoro- and "Coupler 8": Hexanamide, 2-(2,4-bis(1,1-dimethylpropyl)phenoxy)-N-(4-((2,2,3,3,4,4,4-heptafluoro-l-oxobutyl)amino)-3-hydroxyphenyl)-;
(10) one or more interlayers possibly including fine-grained nonsensitized silver halide; and
(11) an antihalation layer.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. 4,366,237; Ep 96,570; U.S. 4,420,556; and U.S. 4,543,323.) Also, the compositions may be blocked or coated in protected form as described, for example, in Japanese Application 61/258,249 or U.S. 5,019,492.

The invention materials may further be used in combination with image-modifying compounds such as "Developer Inhibitor-Releasing" compounds (DIR's). DIR's useful in conjunction with the compositions of the invention are known in the art and examples are described in U.S. Patent Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346, 899; 362, 870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography," C.R. Barr, J.R. Thirtle and P.W. Vittum in Photographic Science and Engineering, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzisodiazoles. In a preferred embodiment, the inhibitor moiety or group is selected from the following formulas: wherein R_{I} is selected from the group consisting of straight and branched alkyls of from 1 to about 8 carbon atoms, benzyl, phenyl, and alkoxy groups and such groups containing none, one or more than one such substituent; R_{II} is selected from R_{I} and -SR_{I}; R_{III} is a straight or branched alkyl group of from 1 to about 5 carbon atoms and m is from 1 to 3; and R_{IV} is selected from the group consisting of hydrogen, halogens and alkoxy, phenyl and carbonamido groups, -COOR_{V} and -NHCOOR_{V} wherein R_{V} is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers).

As mentioned, the developer inhibitor-releasing coupler may include a timing group which produces the time-delayed release of the inhibitor group such as groups utilizing the cleavage reaction of a hemiacetal (U.S. 4,146,396, Japanese Applications 60-249148; 60-249149); groups using an intramolecular nucleophilic substitution reaction (U.S. 4,248,962); groups utilizing an electron transfer reaction along a conjugated system (U.S. 4,409,323; 4,421,845; Japanese Applications 57-188035; 58-98728; 58-209736; 58-209738) groups utilizing ester hydrolysis (German Patent Application (OLS) No. 2,626,315; groups utilizing the cleavage of imino ketals (U.S. 4,546,073); groups that function as a coupler or reducing agent after the coupler reaction (U.S. 4,438,193; U.S. 4,618,571) and groups that combine the features describe above. It is typical that the timing group or moiety is of one of the formulas: wherein IN is the inhibitor moiety, Z is selected from the group consisting of nitro, cyano, alkylsulfonyl; sulfamoyl (-SO₂NR₂); and sulfonamido (-NRSO₂R) groups; n is 0 or 1; and R_{VI} is selected from the group consisting of substituted and unsubstituted alkyl and phenyl groups. The oxygen atom of each timing group is bonded to the coupling-off position of the respective coupler moiety of the DIAR.

Suitable developer inhibitor-releasing couplers for use in the present invention include, but are not limited to, the following:

It is also contemplated that the concepts of the present invention may be employed to obtain reflection color prints as described in Research Disclosure, November 1979, Item 18716, available from Kenneth Mason Publications, Ltd, Dudley Annex, 12a North Street, Emsworth, Hampshire P0101 7DQ, England, incorporated herein by reference. Materials of the invention may be coated on pH adjusted support as described in U.S. 4,917,994; with epoxy solvents (EP 0 164 961); with nickel complex stabilizers (U.S. 4,346,165; U.S. 4,540,653 and U.S. 4,906,559 for example); with ballasted chelating agents such as those in U.S. 4,994,359 to reduce sensitivity to polyvalent cations such as calcium; and with stain reducing compounds such as described in U.S. 5,068,171. Other compounds useful in combination with the invention are disclosed in Japanese Published Applications described in Derwent Abstracts having accession numbers as follows: 90-072,629, 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

Especially useful in this invention are tabular grain silver halide emulsions. Specifically contemplated tabular grain emulsions are those in which greater than 50 percent of the total projected area of the emulsion grains are accounted for by tabular grains having a thickness of less than 0.3 micron (0.5 micron for blue sensitive emulsion) and an average tabularity (T) of greater than 25 (preferably greater than 100), where the term "tabularity" is employed in its art recognized usage as T = ECD/t² where ECD is the average equivalent circular diameter of the tabular grains in microns and t is the average thickness in microns of the tabular grains.

The average useful ECD of photographic emulsions can range up to about 10 microns, although in practice emulsion ECD's seldom exceed about 4 microns. Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim tabular grain projected areas be satisfied by thin (t < 0.2 micron) tabular grains. To achieve the lowest levels of granularity it is preferred that aim tabular grain projected areas be satisfied with ultrathin (t < 0.06 micron) tabular grains. Tabular grain thicknesses typically range down to about 0.02 micron. However, still lower tabular grain thicknesses are contemplated. For example, Daubendiek et al U.S. Patent 4,672,027 reports a 3 mole percent iodide tabular grain silver bromoiodide emulsion having a grain thickness of 0.017 micron.

To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabular grains satisfying the thickness criteria above account for at least 90 percent of total grain projected area.

Suitable tabular grain emulsions can be selected from among a variety of conventional teachings, such as those of the following: Research Disclosure, Item 22534, January 1983, published by Kenneth Mason Publications, Ltd., Emsworth, Hampshire P010 7DD, England; U.S. Patent Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069 and 5,061,616. In addition, use of [100] silver chloride emulsions as described in European patent publication No. 543,395 are specifically contemplated.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

It is understood throughout this specification and claims that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form, but also its form substituted with any photographically useful substituents. Usually the substituent will have less than 30 carbon atoms and typically less than 20 carbon atoms.

The following examples illustrate the invention.

### Preparation of Dispersion 1 (comparative):

A dispersion of the magenta coupler M-1 was prepared in the following manner. 3.4 grams of dibutyl phthalate was heated to 140°C in a heating mantle. 3.4 grams of the coupler was then dissolved in the solvent to constitute the oil phase. The aqueous phase was prepared by combining 44 grams of 11.36% w/w solution of Type IV gelatin in water with 5.0 grams of a 10% w/w solution of the surfactant Alkanol XC™ and 44.2 grams of distilled water at 65°C. The aqueous phase was then combined with the oil phase and the mixture was passed twice through a microfluidizer at 7300 psi to obtain the dispersion.

### Preparation of Dispersion 2 (comparative):

This dispersion was prepared in the same manner as dispersion 1 except that tricresyl phosphate was used in place of dibutyl phthalate.

### Preparation of Dispersion 3 (invention):

1.4 grams of dibutyl phthalate was heated to 140°C in a heating mantle. 3.4 grams of M-1 was added to the solvent followed by 2.0 grams of R-A. The remainder of the procedure was similar to that for Dispersion 1.

### Preparation of Dispersion 4 (comparative):

1.4 grams of dibutyl phthalate was heated to 140°C in a heating mantel. 3.4 grams of M-1 was added to the solvent followed by 12.27 grams of a 16.3% w/w solution of a copolymer of butyl acrylate and acrylic acid (90:10 by weight) in ethyl acetate. The ethyl acetate was allowed to evaporate. The remainder of the procedure was similar to that for Dispersion 1.

The dispersions were combined with emulsion and coated on a paper support. The coating format is shown below. The numbers indicate coverages in g/m².

35 mm strips were obtained from the coatings. The strips were exposed using a 0-3 density 21 step tablet and were processed using the standard RA-4 process. Processed strips from each coating were subjected to 50 Klux high intensity daylight (HID) radiation for five days to determine image stability. Given below is a summary of the fresh Dmax and the change (Δ)in blue density in the Dmin area after five days exposure to 50 Klux HID radiation.

| Dispersion # | | Fresh Dmax | Δ Dmin Blue |
|---|---|---|---|
| 1 | comparative | 2.5 | 0.14 |
| 2 | comparative | 2.5 | 0.17 |
| 3 | invention | 2.4 | 0.04 |
| 4 | comparative | 1.4 | 0.10 |

It is clear that the method of the invention gives good color reproduction and excellent image stability.

### Example 2

This example illustrates the effect of R-A on fading of a magenta image dye.

### Preparation of a Dispersion 5 (comparative):

A dispersion of the magenta image dye Dye 1 was prepared in the following manner. 0.5 grams of dibutyl phthalate was combined with 0.5 grams of Dye 1 and 20 grams of ethyl acetate to constitute the oil phase. The aqueous phase was prepared by combining 32.9 grams of a 11.48% w/w solution of Type IV gelatin in water with 5.0 grams of 10% w/w solution of the surfactant Alkanol XC™ and 50.0 grams of distilled water. The aqueous phase was combined with the oil phase while stirring and the mixture was passed three times through a colloid mill to obtain the dispersion. The ethyl acetate was then removed from the dispersion by evaporation at 60°C and reduced pressure.

### Preparation of Dispersion 6 (invention):

This was prepared in the same manner as Dispersion 5 except that the oil phase was made by combining 0.2 grams of dibutyl phthalate with 0.5 grams of Dye 1, 0.3 grams of R-A and 20 grams of ethyl acetate.

The dispersions were coated on a paper support to give a coverage of 0.1 g/m² of dye. An ultraviolet light protection layer was coated above the layer containing the dye. The coatings were exposed to 50 Klux high intensity daylight radiation and the extent of dye fade was determined. The latter is reported as a percentage of the initial density; i.e. dye fade = {(Di-Df)/Di)x 100 where Di is the initial status A green density and Df is the final density.

| Dispersion # | | Dye Fade |
|---|---|---|
| 5 | comparative | 61.3 |
| 6 | invention | 40.9 |

It is clear that the method of the invention results in a significant improvement in dye fade.

### Example 3

### Preparation of Dispersion 7 (comparative):

A dispersion of the magenta coupler M-1 was prepared in the following manner. 3.4 grams of dibutyl phthalate was heated to 140°C in a heating mantel. 3.4 grams of the coupler was then dissolved in the solvent to constitute the oil phase. The aqueous phase was prepared by combining 44 grams of a 11.36% w/w solution of Type IV gelatin in water with 5 grams of 10% w/w solution of Alkanol XC™ and 44.2 grams of distilled water. The aqueous phase was maintained at 65°C. The aqueous phase was combined with the oil phase and the mixture was passed twice through a microfluidizer at 7200 psi to obtain the dispersion.

### Preparation of Dispersion 8 (comparative):

A dispersion of the magenta coupler M-2 was prepared in the same manner as above except that M-2 was used in place of M-1.

### Preparation of Dispersion 9 (comparative):

A dispersion of the magenta coupler M-3 was prepared in the same manner as Dispersion 7 except that M-3 was used in place of M-1.

### Preparation of Dispersion 10 (invention):

This was prepared in the following manner. 1.7 grams of dibutyl phthalate was heated to 140°C in a heating mantel. 3.4 grams of the coupler M-1 and 1.7 grams of R-A were then dissolved in the solvent to constitute the oil phase. The remainder of the preparation was the same as that described under Dispersion 7.

### Preparation of Dispersion 11 (invention):

This was prepared in the same manner as Dispersion 10 except the M-2 was used in place of M-1.

### Preparation of Dispersion 12 (invention):

This was prepared in the same manner as Dispersion 10 except the M-3 was used in place of M-1.

The dispersions were combined with emulsion and coated on a paper support. The format is shown below. The numbers indicated coverages in g/m².

Unexposed strips based on the above coatings were processed by the standard RA-4 process and then exposed to 50 Klux high intensity daylight radiation for two weeks. The change in Status A blue density was noted.

| Dispersion # | | Δ Blue Density |
|---|---|---|
| 7 | comparative | 0.11 |
| 8 | comparative | 0.04 |
| 9 | comparative | 0.08 |
| 10 | invention | 0.02 |
| 11 | invention | 0.00 |
| 12 | invention | 0.02 |

It is clear that the method of the invention results in significant improvement in photochemical yellowing.

### Example 4

### Preparation of Dispersion 13 (comparative) :

A dispersion of M-1 was prepared in the same manner as dispersion 1 except that tricresylphosphate was used in place of dibutyl phthalate.

### Preparation of Dispersion 14 (invention):

This dispersion was prepared in the same manner as Dispersion 3 except that tricresylphosphate was used in place of dibutyl phthalate.

The dispersions were coated in the same format as described under Example 1. 35 mm strips were obtained from the coatings. Unexposed strips were processed using the standard RA-4 process and then subjected to 50 Klux high intensity daylight (HID) radiation for three days. Given below is the change in status A blue density following exposure to the high density radiation.

| Dispersion # | | Δ Dmin Blue |
|---|---|---|
| 13 | comparative | 0.14 |
| 14 | invention | 0.04 |

Once again the method of the invention gives significant improvement in photochemical yellowing.

## Claims

1. A silver halide colour photographic element comprising at least one light sensitive silver halide emulsion layer comprising a hydrophilic colloid phase and an oily-phase comprising dispersed particles of a ballasted photographic coupler and an organic solvent, characterized in that the oily phase additionally comprises at least one non color forming, oil-soluble, monomeric or oligomeric organic compound having a molecular weight below 1,000 and a glass transition temperature between 0° C and 150°C selected from oil soluble gums, rosins, natural resins and their derivatives, esters of lactose, oil soluble galactomannons, glycol esters, naturally occurring esters of oligomeric glycol esters, alkylbetaglycoside ethers, where the alkyl group contains at least 8 carbon atoms, and water-insoluble derivatives of sucrose, esterified sugars or sugar alcohols esterified with at least four fatty acid groups, and esterified alkoxylated sugars or sugar alcohols esterified with at least four fatty acid groups.

2. A photographic element according to claim 1 comprising a plurality of light sensitive layers including at least one layer sensitive to red light and comprising a silver halide emulsion and a ballasted cyan dye forming coupler, at least one layer sensitive to green light and comprising a silver halide emulsion and a ballasted magenta dye forming coupler and at least one layer sensitive to blue light and comprising a silver halide emulsion and a ballasted yellow dye forming coupler.

3. A photographic element according to claim 1 or 2, wherein said organic compound is selected from the group consisting of oil-soluble gums, rosins, rosin derivatives, natural resins and derivatives thereof, and oil-soluble sucrose derivatives.

4. A photographic element according to claim 3, wherein the organic compound is a rosin derivative of the formula: where A is a saturated or unsaturated alkyl group of 1-10 carbons; B is a hydrogen atom or a saturated or unsaturated alkyl group of 1-10 carbons and n is 0 or 1, and bonds between the numbered corners of the ring structure are single or double bonds,

5. A photographic element according to claim 4, wherein the rosin derivative is abietic acid.

6. A photographic element according to claim 1 comprising at least one layer comprising at least one non-color forming, oil-soluble, monomeric or oligomeric organic compound comprising a sucrose derivative having a glass transition temperature between 0° and 150°C.

7. A photographic element according to claim 6, wherein the organic compound is sucrose octaacetate.

8. A method of improving the image stability of a silver halide color photographic element comprising at least one light sensitive silver halide emulsion layer comprising a hydrophilic colloid phase and an oily-phase comprising dispersed particles of a ballasted photographic coupler and an organic solvent, characterized by incorporating in said oily-phase at least one non color forming, oil-soluble, monomeric or oligomenc organic compound having a molecular weight below 1,000 and a glass transition temperature between 0°C and 150°C selected from oil soluble gums, rosins, natural resins and their derivatives, esters of lactose, oil soluble galactomannons, glycol esters, naturally occurring esters of oligomeric glycol esters, alkylbetaglycoside ethers, where the alkyl group contains at least 8 carbon atoms, and water-insoluble derivatives of sucrose, esterified sugars or sugar alcohols esterified with at least four fatty acid groups, and esterified alkoxylated sugars or sugar alcohols esterified with at least four fatty acid groups.

## Patentansprüche

1. Farbphotographisches Silberhalogenid-Element, umfassend mindestens eine lichtempfindliche Silberhalogenid-Emulsionsschicht, welche eine hydrophile Kolloidphase und eine ölige Phase umfaßt, die dispergierte Teilchen eines mit Ballastgruppen versehenen photographischen Kupplers und ein organisches Lösungsmittel umfaßt, dadurch gekennzeichnet, daß die ölige Phase zusätzlich mindestens eine keine Farbe bildende, öllösliche, monomere oder oligomere organische Verbindung mit einem Molekulargewicht unterhalb von 1000 und einer Glasübergangstemperatur zwischen 0°C und 150°C umfaßt, welche aus öllöslichen Gummis, Kolophonium, natürlichen Harzen und deren Derivaten, Estern von Lactose, öllöslichen Galactomannanen, Glycolestern, natürlich vorkommenden Estern von oligomeren Glycolestern, Alkyl-beta-glycosidethern, worin die Alkylgruppe mindestens 8 Kohlenstoffatome enthält, und in Wasser unlöslichen Derivaten von Saccharose, veresterten Zuckern oder Zuckeralkoholen, die mit mindestens vier Fettsäuregruppen verestert sind, und veresterten alkoxylierten Zuckern oder Zuckeralkoholen, die mit mindestens vier Fettsäuregruppen verestert sind, ausgewählt ist.

2. Photographisches Element nach Anspruch 1, umfassend eine Mehrzahl von lichtempfindlichen Schichten, die mindestens eine Schicht, die für rotes Licht empfindlich ist und eine Silberhalogenidemulsion und einen mit einer Ballastgruppe versehenen Cyanfarbstoff bildenden Kuppler umfaßt, mindestens eine Schicht, die für grünes Licht empfindlich ist und eine Silberhalogenidemulsion und einen mit einer Ballastgruppe versehenen Magentafarbstoff bildenden Kuppler umfaßt, und mindestens eine Schicht, die für blaues Licht empfindlich ist und eine Silberhalogenidemulsion und einen mit einer Ballastgruppe versehenen gelben Farbstoff bildenden Kuppler umfaßt, einschließen.

3. Photographisches Element nach Anspruch 1 oder 2, in welchem die organische Verbindung aus der Gruppe ausgewählt ist, die aus öllöslichen Gummis, Kolophonium, Kolophonium-Derivaten, natürlichen Harzen und deren Derivaten und öllöslichen Saccharose-Derivaten besteht.

4. Photographisches Element nach Anspruch 3, in welchem die organische Verbindung ein Kolophonium-Derivat der Formel: ist, in der A eine gesättigte oder ungesättigte Alkylgruppe mit 1 - 10 Kohlenstoffen ist; B ein Wasserstoffatom oder eine gesättigte oder ungesättigte Alkylgruppe mit 1 - 10 Kohlenstoffen ist und n für 0 oder 1 steht und Bindungen zwischen den numerierten Ecken der Ringstruktur Einfach- oder Doppelbindungen sind.

5. Photographisches Element nach Anspruch 4, in welchem das Kolophonium-Derivat Abietinsäure ist.

6. Photographisches Element nach Anspruch 1, umfassend mindestens eine Schicht, die mindestens eine keine Farbe bildende, öllösliche, monomere oder oligomere organische Verbindung umfaßt, welche ein Saccharose-Derivat mit einer Glasübergangstemperatur zwischen 0 und 150°C umfaßt.

7. Photographisches Element nach Anspruch 6, in welchem die organische Verbindung Saccharoseoctaacetat ist.

8. Verfahren zur Verbesserung der Bildstabilität eines farbphotographischen Silberhalogenid-Elementes, das mindestens eine lichtempfindliche Silberhalogenid-Emulsionsschicht umfaßt, welche eine hydrophile Kolloidphase und eine ölige Phase umfaßt, die dispergierte Teilchen eines mit einer Ballastgruppe versehenen photographischen Kupplers und ein organisches Lösungsmittel umfaßt, dadurch gekennzeichnet, daß man der Ölphase mindestens eine keine Farbe bildende, öllösliche, monomere oder oligomere organische Verbindung mit einem Molekulargewicht unterhalb von 1000 und einer Glasübergangstemperatur zwischen 0°C und 150°C einverleibt, welche aus öllöslichen Gummis, Kolophonium, natürlichen Harzen und deren Derivaten, Estern von Lactose, öllöslichen Galactomannanen, Glycolestern, natürlich vorkommenden Estern von oligomeren Glycolestern, Alkyl-betaglycosidethern, worin die Alkylgruppe mindestens 8 Kohlenstoffatome enthält, und in Wasser unlöslichen Derivaten von Saccharose, veresterten Zuckern oder Zuckeralkoholen, die mit mindestens vier Fettsäuregruppen verestert sind, und veresterten alkoxylierten Zuckern oder Zuckeralkoholen, die mit mindestens vier Fettsäuregruppen verestert sind, ausgewählt ist.

## Revendications

1. Elément photographique en couleurs aux halogénures d'argent contenant au moins une couche d'émulsion aux halogénures d'argent sensible à la lumière comprenant une phase de colloïde hydrophile et une phase huileuse comprenant des particules dispersées d'un coupleur photographique ballasté et d'un solvant organique, caractérisé en ce que la phase huileuse comprend en outre au moins un composé organique, oligomère ou monomère soluble dans l'huile, non chromogène, ayant un poids moléculaire inférieur à 1 000 et une température de transition vitreuse comprise entre 0°C et 150°C, choisi parmi les gommes, les colophanes, les résines naturelles solubles dans l'huile et leurs dérivés, les esters de lactose, les galactomannons solubles dans l'huile, les esters de glycol, les esters naturels des esters de glycol oligomères, les éthers alkylbétaglycoside, où le groupe alkyle contient au moins 8 atomes de carbone et des dérivés du sucrose insolubles dans l'eau, des sucres estérifiés ou des alcools sacchariques estérifiés par au moins quatre groupes acides gras et des sucres estérifiés alcoxylés ou des alcools sacchariques estérifiés par au moins quatre groupes acides gras.

2. Elément photographique selon la revendication 1 contenant une pluralité de couches sensibles à la lumière, y compris au moins une couche sensible à la lumière rouge et comprenant une émulsion aux halogénures d'argent et un coupleur formateur de colorant cyan ballasté, au moins une couche sensible à la lumière verte et comprenant une émulsion aux halogénures d'argent et un coupleur formateur de colorant magenta et au moins une couche sensible à la lumière bleue et comprenant une émulsion aux halogénures d'argent et un coupleur formateur de colorant jaune ballasté.

3. Elément photographique selon la revendication 1 ou 2, dans lequel ledit composé organique est choisi parmi le groupe comprenant les gommes, les colophanes, les dérivés de la colophane, les résines naturelles solubles dans l'huile et les dérivés de ces dernières ainsi que les dérivés du sucrose solubles dans l'huile.

4. Elément photographique selon la revendication 3, dans lequel le composé organique est un dérivé de la colophane représenté par la formule : où A est un groupe alkyle saturé ou insaturé de 1 à 10 atomes de carbone ; B est un atome d'hydrogène ou un groupe alkyle saturé ou insaturé de 1 à 10 atomes de carbone et n est 0 ou 1, et où les liaisons entre les deux coins numérotés de la structure cyclique sont des liaisons simples ou doubles.

5. Elément photographique selon la revendication 4, dans lequel le dérivé de la colophane est l'acide abiétique.

6. Elément photographique selon la revendication 1 comprenant au moins une couche contenant au moins un composé organique, oligomère ou monomère, soluble dans l'huile, non chromogène, comprenant un dérivé du sucrose ayant une température de transition vitreuse comprise entre 0°C et 150°C.

7. Elément photographique selon la revendication 6, dans lequel le composé organique est l'octaacétate de sucrose.

8. Procédé permettant d'améliorer la stabilité de l'image d'un élément photographique en couleurs aux halogénures d'argent comprenant au moins une couche d'émulsion aux halogénures d'argent sensible à la lumière comprenant une phase de colloïde hydrophile et une phase huileuse comprenant des particules dispersées d'un coupleur photographique ballasté et d'un solvant organique, caractérisé en ce que l'on incorpore dans ladite phase huileuse au moins un composé organique, oligomère ou monomère, soluble dans l'huile, non chromogène, ayant un poids moléculaire inférieur à 1 000 et une température de transition vitreuse comprise entre 0°C et 150°C, choisi parmi les gommes, les colophanes, les résines naturelles solubles dans l'huile et leurs dérivés, les esters de lactose. les galactomannons solubles dans l'huile, les esters de glycol, les esters naturels des esters de glycol oligomères, les éthers alkylbétaglycoside, où le groupe alkyle contient au moins 8 atomes de carbone et des dérivés du sucrose insolubles dans l'eau, des sucres estérifiés ou des alcools sacchariques estérifiés par au moins quatre groupes acides gras et des sucres estérifiés alcoxylés ou des alcools sacchariques estérifiés par au moins quatre groupes acides gras.
